

## UNITED STATES PATENT OFFICE

2,336,070

## LUBRICATING OIL

Richard G. Clarkson, Wilmington, Del., assignor  
to E. I. du Pont de Nemours & Company, Wil-  
mington, Del., a corporation of Delaware

No Drawing. Application September 18, 1942,  
Serial No. 458,823

12 Claims. (Cl. 252—51)

This invention relates to lubricating oils and more particularly to lubricating oils which contain or tend to form sludge and also contain compounds to inhibit the separation of insoluble sludge from the oils.

Lubricating oils deteriorate under the conditions to which they are exposed in internal combustion engines. This deterioration is accompanied by the formation of organic acids and by the separation of insoluble sludge. The organic acids tend to corrode alloy bearings, and the insoluble sludge which separates fouls the internal surfaces of the engine. Eventually, as more sludge separates, the oil lines become clogged and delivery of the oil to moving parts is prevented, with resultant engine failure. Various agents have been suggested which, it is claimed, will lengthen the period of useful service of a lubricating oil before harmful deterioration becomes evident. Other agents have been suggested which, it is claimed, will protect alloy bearings against corrosion by organic acids. In compounding heavy-duty lubricating oils, especially for Diesel engines, it has recently been found desirable to add compounds which have detergent and dispersive properties. Such compounds tend to prevent the fouling of engine parts and filters, and result in much cleaner engines. They are believed to maintain the sludge, formed as the oil deteriorates, in a state of colloidal dispersion. In some cases, they display sufficient detergent action to remove existing deposits from a previously fouled engine. A number of compounds, which are claimed to display detergent and dispersive properties, have been disclosed in the prior art. These compounds are all organo-metallic compounds of various types and in general have been found to accelerate corrosion of alloy bearings. (S. A. E. Transactions, April, 1941, pages 128-137 "Crankcase Oils for Heavy Duty Service," by H. R. Wolf).

It is an object of the present invention to provide lubricating oils having a materially decreased tendency to separate and deposit sludge. Another object is to treat lubricating oils, normally tending to deposit insoluble sludge, to inhibit the separation and deposition of the insoluble sludge. A further object is to provide a method for inhibiting the deposition of sludge on an internal combustion engine during operation thereof. A 50

still further object is to provide lubricating oils which are particularly adapted for use in heavy-duty service over longer periods of time in an internal combustion engine with less fouling of the engine. Other objects are to provide new compositions of matter. Still other objects will appear hereinafter.

The above and other objects may be accomplished in accordance with my invention which 10 comprises incorporating in a mineral lubricating oil, normally tending to separate and deposit insoluble sludge, a small proportion of an acylated polyamine containing at least 14 carbon atoms in which each acyl group is derived from a naphthenic acid and the polyamine group is derived from an aliphatic polyamine containing at least 2 primary amino groups separated by at least 2 carbon atoms. I have found that such acylated polyamines are very effective for preventing the 15 separation of insoluble sludge from lubricating oils, being more effective than compounds which have heretofore been proposed for this purpose. In addition, such acylated polyamines do not have any tendency to promote the corrosion of sensitive bearing metals and hence my compounds do 20 not have the disadvantageous properties of the compounds heretofore proposed for this purpose.

The oils, to which the acylated polyamines are 25 to be added in accordance with my invention, are the usual mineral lubricating oils which normally tend to form sludge in service or which may even contain sludge already formed. My invention is particularly concerned with the treatment of petroleum lubricating oils employed in heavy-duty 30 service where the tendency for the oils to form insoluble sludge and for such sludge to deposit upon and foul the engines is particularly severe.

The acylated polyamines, which are to be employed in accordance with my invention, may be 35 represented by the general formula



45 wherein A represents a naphthenic acid acyl group, B represents hydrogen or a naphthenic acid acyl group, X is an aliphatic group containing at least two carbon atoms and A-X+B contain a total of at least 14 carbon atoms. The two nitrogens in the formula are bonded to

separate carbon atoms in the aliphatic group represented by  $\text{X}$ .

The acyl group or groups are derived from naphthenic acids. The naphthenic acids occur naturally in crude petroleum and are usually obtained therefrom in the form of mixtures of acids of different molecular weights. They are cyclic, generally containing a five-membered carbocyclic ring with the carboxyl group mainly on the end of an alkyl side chain. They are distinguished from the natural fatty acids and the fatty acids, obtained by the oxidation of paraffin wax and the like, in that such products are open chain carboxylic acids.

Amides, wherein the acyl groups are derived from the open chain fatty acids, are soluble in lubricating oils to a very limited extent only. On the other hand, the acylated polyamines or amides of my invention, in which the acyl groups are derived from naphthenic acids, are quite soluble in lubricating oils and can be readily dissolved in the oils in the amounts desired. Therefore, I generally prefer to employ the amides derived from the naphthenic acids. By the term "naphthenic acid," I mean those derived from petroleum. The naphthenic acids are ordinarily obtained as mixtures and appear on the market as such. Such commercial mixtures of naphthenic acids are particularly desirable for preparing the acylated polyamines to be employed in accordance with my invention.

The polyamine group in the acylated polyamines or amides, which may be employed in accordance with my invention, may be derived from any open chain aliphatic polyamine containing at least two primary amino groups separated by at least two carbon atoms. The polyamine group may be represented by the formula



wherein the two nitrogens represent the nitrogens of the two primary amino groups and  $\text{X}$  represents an open chain divalent aliphatic group of at least two carbon atoms. The aliphatic chain may contain internal linkages such as  $-\text{O}-$ ,  $-\text{S}-$ ,  $-\text{S}-\text{S}-$ ,  $-\text{SO}-$ ,  $-\text{SO}_2-$ ,  $-\text{NH}-$  and  $-\text{NR}-$  wherein  $\text{R}$  represents an aliphatic group or a naphthenic acid acyl group. Preferably, the polyamine group is derived from an alkylene polyamine and, particularly, from an alkylene diamine. By the terms "alkylene polyamine" and "alkylene diamine," I mean that such polyamines or diamines consist of the elements carbon, hydrogen and nitrogen solely, the nitrogen being present in amino groups. Also preferably, the two primary amino groups are separated by only two carbon atoms as in ethylene diamine, 1,2-propylene diamine and 2,3-butylene diamine. Particularly suitable acylated polyamines have been prepared from

- (1) Ethylene diamine,  $\text{H}_2\text{NCH}_2\text{CH}_2\text{NH}_2$ ,
- (2) 1,2-propylene diamine,  $\text{H}_2\text{NCH}_2\text{CH}_2\text{NH}_2$ ,
- (3) Hexamethylene diamine,  $\text{H}_2\text{NCH}_2\text{CH}_2\text{CH}_2\text{CH}_2\text{CH}_2\text{CH}_2\text{NH}_2$ ,
- (4) Diethylene triamine,  $\text{H}_2\text{NCH}_2\text{CH}_2\text{NHCH}_2\text{CH}_2\text{NH}_2$ ,
- (5) Triethylene tetra-  
mine,  $\text{H}_2\text{NCH}_2\text{CH}_2\text{NHCH}_2\text{CH}_2\text{NHCH}_2\text{CH}_2\text{NH}_2$ ,
- (6) Di-( $\gamma$ -amino propyl)-  
methyl amine,  $\text{H}_2\text{NCH}_2\text{CH}_2\text{CH}_2\text{NCH}_2\text{CH}_2\text{CH}_2\text{NH}_2$ ,
- (7) Di-( $\beta$ -amino ethyl)-sulfide,  $\text{H}_2\text{NCH}_2\text{CH}_2\text{SCH}_2\text{CH}_2\text{NH}_2$ ,

Other polyamines, which may be employed for producing suitable acylated polyamines, are—



The acylated polyamines, which are to be employed in accordance with my invention, may contain one or more acyl groups for each polyamine group. Preferably, I employ the polyacylated polyamines wherein there is one acyl group for each primary amino group of the polyamine. I particularly prefer the diacylated diamines. Of these, the most effective and desirable appear to be the di-naphthenic amides of ethylene diamine and the di-naphthenic amides of 1,2-propylene diamine.

The amounts of the acylated polyamines will vary greatly depending upon the effectiveness of the particular amide and on the amount of sludge in the oil and the amount of sludge normally formed by the oil under the particular conditions under which it is to be employed. Usually, the amide will be employed within the range of from about 0.1% to about 5% by weight based on the oil. Larger amounts may be necessary in extreme cases.

The acylated polyamines or amides of my invention may be prepared by the action of the naphthenic acid, its halide, nitrile or ester on the polyamine, by methods which are well known to the art. The preferred method involves mixing the theoretical equivalents of acid and amine and heating to from about 180° C. to about 190° C. under an atmosphere of nitrogen until the theoretical amount of water has distilled out. The crude reaction mixtures, as thus obtained, are quite suitable for use in accordance with my invention without separating or purifying the amide.

The following test has been devised to allow rapid evaluation of sludge dispersant properties of various addition agents in oils.

A 75 cc. sample of commercial S. A. E. 20 oil, containing a definite concentration of the additive being tested and 2.0% of naphthenic acids, was heated to 150° C. Two ccs. of a benzene soluble sludge extract were added and the solution was stirred for two minutes.

A 45 gram sample of the sludge-oil mixture was weighed into a 100 cc. centrifuge tube and, after cooling to room temperature, 50 ccs. of A. S. T. M. naphtha were added, the tube stoppered and shaken, and then centrifuged 45 minutes. The volume of separated sludge was observed and recorded. In each set of tests, one sample of control oil, containing naphthenic acid and sludge but no dispersant additive, was included. The efficiency of a given additive as a

sludge dispersant was calculated from the formula:

$$\% \text{ dispersion} = \frac{\text{cc. sludge control} - \text{cc. sludge test}}{\text{cc. sludge control}}$$

The purpose of the naphthenic acid in the test was to simulate the conditions in a partially oxidized oil in which organic acids are present. The addition of the benzene solution of sludge to the hot oil roughly duplicates the formation of sludge in an oil in use. The purpose of the dilution with A. S. T. M. naphtha is to reduce the viscosity of the medium in order to permit effective separation of sludge by centrifuging.

The following table illustrates the effective dispersion of sludge in oil containing compounds of our invention.

Table I

| Additive, amide from—                         |                 | Ratio | Conc. of additive in oil | Percent dispersion of added sludge |
|-----------------------------------------------|-----------------|-------|--------------------------|------------------------------------|
| Amine                                         | Acid            |       |                          |                                    |
| Ethylene diamine.....                         | Naphthenic..... | 1:2   | 2                        | 85-98                              |
| .....                                         | .....           | ..... | 1                        | 72-90                              |
| .....                                         | .....           | ..... | .5                       | 40-76                              |
| .....                                         | .....           | ..... | .25                      | 32-33                              |
| 1,2-propylene diamine.....                    | .....do.....    | 1:2   | 2                        | 60-96                              |
| .....                                         | .....do.....    | ..... | 1                        | 44-88                              |
| .....                                         | .....do.....    | ..... | .5                       | 44-87                              |
| Hexamethylene diamine.....                    | .....do.....    | 1:2   | 2                        | 73-74                              |
| .....                                         | .....do.....    | ..... | 1                        | 52                                 |
| Diethylene triamine.....                      | .....do.....    | 1:1   | .5                       | 8                                  |
| Do.....                                       | .....do.....    | 1:2   | 2                        | 50                                 |
| Do.....                                       | .....do.....    | 1:3   | 2                        | 84                                 |
| Triethylene tetraamine.....                   | .....do.....    | 1:2   | 2                        | 79                                 |
| Do.....                                       | .....do.....    | 1:4   | 2                        | 81                                 |
| Di-( $\gamma$ -aminopropyl)-methyl amine..... | .....do.....    | 1:2   | 2                        | 87                                 |
| Di-( $\beta$ -aminoethyl)-sulfide.....        | .....do.....    | 1:2   | 2                        | 53                                 |
| .....                                         | .....do.....    | 1:2   | 2                        | 72                                 |

<sup>1</sup> Part of naphthenic acid may not have formed amide but only ammonium soap.

In the above table, the numbers, under ratio, indicate that the amides employed were those obtained from 1, 2, 3 and 4 moles of the acid and 1 mole of the polyamine. The naphthenic acid amides were prepared from a commercial refined mixture of naphthenic acids having an acid number of 230-240 and was composed of naphthenic acids having an average number of carbon atoms calculated as approximately 15. Such naphthenic acid amides are oily substances having a high degree of solubility in petroleum oils. Another naphthenic acid amide was prepared from 1 mole of 1,2-propylene diamine and 2 moles of a commercial mixture of refined naphthenic acids having an acid number of 125 and an apparent average of approximately 30 carbon atoms. This last compound, when subjected to the above test in 2% concentration in the oil, gave a 60% dispersion of the sludge.

The acylated polyamines or amides of my invention have no substantial pour depressant properties. This is illustrated by the results of tests given in the following Table II:

Table II

[The base oil, used for determining pour depressant effect in these tests, had a pour of +20° F.]

| Compound, amide from—                      | Ratio | Pour point, ° F. |    |
|--------------------------------------------|-------|------------------|----|
|                                            |       | 2%               | 5% |
| Naphthenic acid, ethylenediamine.....      | 2:1   | 20               | 20 |
| Naphthenic acid, diethylenetriamine.....   | 2:1   | 20               | 15 |
| Naphthenic acid, triethylenetetramine..... | 2:1   | 20               | 15 |

It will be understood that the specific embodiments disclosed hereinbefore and the tests thereon are given for illustrative purposes only. It will be apparent that many variations and modifications can be made in the compounds and the conditions and proportions employed without departing from the spirit or scope of my invention. The oil compositions may contain other addition agents which perform other functions, such as pour point depressants, corrosion inhibitors, oiliness agents, extreme pressure agents and the like. Accordingly, I intend to cover my invention broadly as in the appended claims.

I claim:

1. A lubricant comprising a mineral lubricating oil, normally tending to separate and deposit insoluble sludge, and a small proportion, sufficient to inhibit deposition of the sludge, of an acylated polyamine containing at least 14 carbon atoms in which each acyl group is derived from a naphthenic acid and the polyamine group is derived from an aliphatic polyamine containing at least two primary amino groups separated by at least 2 carbon atoms.
2. A lubricant comprising a mineral lubricating oil, normally tending to separate and deposit insoluble sludge, and a small proportion, sufficient to inhibit deposition of the sludge, of an acylated polyamine containing at least 14 carbon atoms in which each acyl group is derived from a naphthenic acid and the polyamine group is derived from an alkylene polyamine containing at least two primary amino groups separated by at least 2 carbon atoms.
3. A lubricant comprising a mineral lubricating oil, normally tending to separate and deposit insoluble sludge, and a small proportion, sufficient to inhibit deposition of the sludge, of an acylated diamine containing at least 14 carbon atoms in which each acyl group is derived from a naphthenic acid and the diamine group is derived from an aliphatic diamine containing two primary amino groups separated by at least 2 carbon atoms.
4. A lubricant comprising a mineral lubricating oil, normally tending to separate and deposit insoluble sludge, and a small proportion, sufficient to inhibit deposition of the sludge, of an acylated diamine containing at least 14 carbon atoms in which each acyl group is derived from a naphthenic acid and the diamine group is derived from an alkylene diamine containing two primary amino groups separated by only 2 carbon atoms.
5. A lubricant comprising a mineral lubricating oil, normally tending to separate and deposit insoluble sludge, and a small proportion, sufficient to inhibit deposition of the sludge, of an acylated ethylene diamine containing at least 14 carbon atoms in which each acyl group is derived from a naphthenic acid and the diamine group is derived from ethylene diamine.
6. A lubricant comprising a mineral lubricating oil, normally tending to separate and deposit insoluble sludge, and a small proportion, sufficient to inhibit deposition of the sludge, of an acylated propylene diamine containing at least 14 carbon atoms in which each acyl group is derived from a naphthenic acid and the diamine group is derived from 1,2-propylene diamine.
7. A lubricant comprising a mineral lubricating oil, normally tending to separate and deposit insoluble sludge, and a small proportion, sufficient to inhibit deposition of the sludge, of a polyacylated polyamine containing at least 14

carbon atoms in which each acyl group is derived from a naphthenic acid and the polyamine group is derived from an aliphatic polyamine containing at least two primary amino groups separated by at least 2 carbon atoms.

8. A lubricant comprising a mineral lubricating oil, normally tending to separate and deposit insoluble sludge, and a small proportion, sufficient to inhibit deposition of the sludge, of a diacylated diamine containing at least 14 carbon atoms in which each acyl group is derived from a naphthenic acid and the diamine group is derived from an aliphatic diamine containing two primary amino groups separated by at least 2 carbon atoms.

9. A lubricant comprising a mineral lubricating oil, normally tending to separate and deposit insoluble sludge, and a small proportion, sufficient to inhibit deposition of the sludge, of a diacylated diamine containing at least 14 carbon atoms in which each acyl group is derived from a naphthenic acid and the diamine group is derived from an alkylene diamine containing two primary amino groups separated by at least 2 carbon atoms.

10. A lubricant comprising a mineral lubricat-

ing oil, normally tending to separate and deposit insoluble sludge, and a small proportion, sufficient to inhibit deposition of the sludge, of a diacylated ethylene diamine containing at least

5 14 carbon atoms in which each acyl group is derived from a naphthenic acid and the diamine group is derived from ethylene diamine.

11. A lubricant comprising a mineral lubricating oil, normally tending to separate and deposit insoluble sludge, and a small proportion, sufficient to inhibit deposition of the sludge, of a diacylated propylene diamine containing at least 14 carbon atoms in which each acyl group is derived from a naphthenic acid and the diamine group is derived from 1,2-propylene diamine.

12. A lubricant comprising a mineral lubricating oil, normally tending to separate and deposit insoluble sludge, and a small proportion, sufficient to inhibit deposition of the sludge, of a diacylated triethylene tetramine containing at least 14 carbon atoms in which each acyl group is derived from a naphthenic acid and the amine group is derived from triethylene tetramine.